

July 7, 1964

E. BERSET

3,140,331

MANUFACTURE OF TILE FOR ACOUSTIC AND DECORATIVE EFFECTS

Filed April 1, 1959



*Fig. 1*



*Fig. 2*

*Fig. 3*



*Fig. 5*



*Fig. 4*

INVENTOR.  
*Edward Berset*  
BY  
*W. Barrett Jones*  
Attorney

**1**

3,140,331

**MANUFACTURE OF TILE FOR ACOUSTIC AND DECORATIVE EFFECTS**

Edward Berset, Cloquet, Minn., assignor to Wood Conversion Company, St. Paul, Minn., a corporation of Delaware

Filed Apr. 1, 1959, Ser. No. 803,523  
4 Claims. (Cl. 264—293)

The present invention relates to the production of tile from felted fiber panel, and in particular to processes for treating the tile face, either for acoustic purposes, or for decorative effect, or both.

Such tile is commonly provided in squares, cut from larger panels which are produced by felting an aqueous slurry of vegetable fibers, for example, on a Fourdrinier machine. Wet felts are pressed and dried. The processing produces various stresses in the dry panel. When the panel is cut into smaller squares some stresses are released. As a result, many tile squares have varying perceptible warp.

The final tile is coated usually by coating the panel before the tile is cut from it. The coat may be applied in whole or in part to the pressed wet felt before drying, or in whole or in part to the panel after pressing the wet felt and drying. In some operations, a prime coat is applied to the pressed wet felt, and after drying, a top coat is applied. The coat and the coating process also introduce stresses leading to perceptible warp. Special treatments in processing the panel may be practiced to insure a predetermined direction of warp such that subsequent processing of tile cut from the panel tend to correct the warp.

Acoustic tile of numerous well-known brands having vegetable fiber bodies, is made by drilling or punching a multiplicity of holes into dry coated tile, in a regular pattern, or in a random pattern, and in each case with holes of uniform size or different sizes. It has been observed that the drilling or punching process as heretofore practiced changed the stress patterns within the tile and this also contributes to warp. When this processing leads to negative warp, which is a dishing of the exposable face, the panel may be processed to introduce positive warp in the tile square cut from it, in order to decrease or eliminate the positive warp by processing the tile.

Other forms of tile are produced for decorative purposes by impressing design patterns into a final coated tile or uncoated tile, or prime-coated tile. Coating material may be applied after the design is impressed. Hot platens and steam or moisture are commonly used to soften the board or coat, or both, thereby to facilitate the impressing action as well as to avoid breaking or cracking an applied coat at certain critical boundaries of the design areas. These operations of impressing, and of coating after impressing also pertain to stresses leading to warp.

The processing of tile as above described constitutes substantially uniform loading of pressure on the exposable face. For acoustical tile this is effected by the numerous drills or punches applied over substantially the entire face of the tile. In the case of tile with impressed designs, it is the pressing platen which applies the load.

Whether the tiles to be processed are unwarped or warped, the processing described tends to produce a negative warp, of which the direction of warp is such as to

**2**

cup or dish the exposable processed face of the tile. Although the warp in a single tile may be almost imperceptible, a ceiling assembly of tiles inevitably evidences that warp when viewed at certain angles to receive reflections from one or more sources of light which are more or less pin-pointed. The more nearly planar all the tile are made, the better a ceiling assembly will be.

In studying the various decorative and acoustic tile above referred to, it was observed that the tile blanks to be processed are placed with the back side on a flat platen. In processing, the face is substantially uniformly loaded and compressed toward said platen. This results in compression of the tile between its faces. If the tile blank to be processed is already warped to a dished face, such compression merely flattens it temporarily. But, during the compression other changes take place. The holes formed cut through material of the panel and any coat thereon and over the area of the hole release any stress of tension or compression. Especially when the holes terminate within the panel, the change in stress is more limited to the face than to the back of the tile. Thus, an originally warped or planar tile blank acquires a tendency to warp negatively merely by forming holes therein for acoustic purposes.

In the case of impressing designs in the tile face, the back has heretofore been placed on a flat platen, and a die-plate embossed with a negative of the pattern is pressed onto the tile to leave an impression. The operation is best performed with a heated plate, which is effective on heat-softenable coats. Moisture in the form of water or steam also facilitates the process. The moisture may soften both the coat and the fibers of the body with or without a surface coat. These factors of mechanical pressure varying with the pattern, the moisture and the heat, change old stresses and introduce new stresses, leading to warping of the tile to a dished face.

The present invention aims to introduce new and anti-warping stresses in a finished tile by certain straining of the tile.

Accordingly, it is an object of the invention so to strain a tile that the warping tendencies of original stresses are modified or eliminated and that new stresses are introduced tending to hold the finished tile in a generally flat condition.

It is a particular object so to strain the tile during the processing of the face as above referred to.

Various other and ancillary objects and advantages of the invention will appear from the following description and expalanation given in connection with the accompanying drawing, in which:

FIG. 1 illustrates partly in cross-section and in perspective, a tile positioned for processing between a support and a pressing member.

FIGS. 2 and 3 represent two pyramidal inserts for supporting the backs of tile processed at the face.

FIG. 4 is a stepped pyramid of concentric squares.

FIG. 5 is an enlarged fragmentary cross-section taken on line 5—5 of FIG. 4.

In carrying out the invention the back of the tile is placed on a supporting platen which is slightly crowned centrally so as to be high in the center with its four edges similarly at a lower level or levels, thus to effect a dished contour on the back face of a tile while compressed onto the platen by any type of substantially uniform loading of the face. The crowned platen is preferably symmetrical

with respect to two right-angular axes, as when it is spherically convex, pyramidal with sides in number which is 4 or a multiple of 4, or a pile of so-centered polygons of thin sheets reducing in size and having sides in number which is 4 or a multiple thereof. Minor departures from such regularity are permissible so long as a generally uniform crowning exists.

Without need to change the hole-forming operation or the design-impressing action, the tile is pressed onto the crowned platen by means at the face, which pressing may be a planar or embossed platen or a bank of drills or punches. As a result, the back of the tile during such compression is dished to match the crowned platen, by thinning the tile at the center more than at its edges. The stresses thus introduced and retained on release of the tile from the operating compression, counter the tendencies to warp the face into slightly dished form.

The following exemplifies conditions heretofore encountered with a coated wood fiber tile 12-inches square,  $\frac{1}{2}$ -inch thick, and with a density of 17 lbs. per cu. ft. When drilling 319 holes into it using hollow drills  $\frac{3}{16}$ -inch or  $\frac{1}{4}$ -inch in diameter, or the two sizes mixed, it has been found that the entrance pressure and the drilling pressure per drill are high, as shown in Table I.

Table I

| Drill Diameter            | Pressure in Pounds Per Drill |          |
|---------------------------|------------------------------|----------|
|                           | Entrance                     | Drilling |
| $\frac{3}{16}$ -inch..... | 11 to 20                     | 6 to 16  |
| $\frac{1}{4}$ -inch.....  | 15 to 32                     | 12 to 26 |

With over 300 drills, the total pressure is very high but distributed and centered at many local areas. This operation carried out as described on a planar supporting platen creates on release a dished warp in the face with the tile center inwardly from the boundary of its edges by an amount varying in the range from .015 to .025 inch.

In the debossing operation above described, the results vary with numerous factors, including the design and its local areas, the depth of design components, the platen pressure and temperature, the coat if any, and the amount of moisture if any.

Because titles vary in the degree of warp from one to another even when cut from the same panel, coated or not, the invention contemplates reducing the tendency of all the tile by similarly processing them, it being understood that perfection to that end result can be effected in some cases. In consequence, the crowning of the supporting platen is fixed at that which produces satisfactory average results for each type of panel material.

It has been found that with the wood fiber panel above described, a given crowning of a supporting platen is satisfactory in both a drilling or punching operation of the kind described, and in a hot-debossing operation as described.

To achieve the desired result, and to practice the invention, an insert which is flat on one face and crowned on the other is placed on the flat supporting platen heretofore used.

In the drawing, the numeral 10 represents a flat supporting platen, such as used heretofore to receive the tile, on which is placed a plano-convex insert 11. A guiding frame for locating the tile is illustrated by the cross-section of three of its members 12, 13 and 14. The tile 15 is shown in the frame. The dotted line block 16 above the tile represents the pressing element or operation being either a planar platen, or a bank of drills or punches or a platen with an embossed negative of a design. Arrow 17 represents movement of plate 16.

With reference to a 12-inch square tile, as described, a satisfactory insert platen is one 15-inches square, with

5 plane face 18, spherically convex face 19, with edges 0.020-inch at maximum thickness, and center 0.085-inch thick, resulting in a differential of 0.065-inch for the insert, nearly all of which is applied to the tile in process.

FIG. 2 shows a pyramidal insert 21 of four similar sides 22. When the center crowning is the same as described for insert 11 it may be substituted for insert 11.

FIGS. 3 and 4 show substitute inserts of the same degree of crowning. FIG. 3 shows a pyramid 24 of eight similar sides 25.

FIG. 4 shows an insert 26 of concentric squares of upwardly decreasing size to effect the desired crowning. It has the thicker base 27, and on its four thin layers 28 to 31 of approximately .016-inch thickness. The base 27 may be wood, hardboard or metal. The layers 28 to 31 may be metal or fiber sheets, the latter being preferred so that the indicated exposed square edges 32 (FIG. 5) thereof may be rounded off as indicated to avoid ridge marks in the back if desired.

In other words, by the present invention the tile is so stressed that in the release of stresses, the movement may still be in the direction to dish the face of the tile, but the movement is from a reverse of the undesired condition so as to stop in the vicinity of the desired planar form, rather than movement away from a planar form into undesired warp.

As examples of debossing designs in tile, see design patents Des. 183,531, and Des. 183,697. The drilling and the debossing alter the stresses in the face. The debossing of designs moves portions of the face to inward locations such that on release of the compression inward locations remain.

I claim:

1. The method of treating a substantially square tile 35 of porous fiberboard useful as ceiling tile, which comprises compressing the tile onto a centrally crowned supporting platen by applying a substantially planar platen and thereby substantially uniformly loading the exposable tile face, whereby during compression to deform the tile to a dished back surface corresponding generally to said crowned platen and thereby altering the original stresses in the uncompressed tile and introducing new stresses in the compressed tile, and releasing the tile from said compression.

2. The method of treating a substantially square tile

50 of porous fiberboard useful as ceiling tile, which comprises compressing the tile onto a centrally crowned supporting platen by applying a heated substantially planar platen embossed with a design and thereby hot-pressing portions of the surface to inward locations and thereby substantially uniformly loading the exposable tile face, whereby during compression to deform the tile to a dished back surface corresponding generally to said crowned platen and thereby altering the original stresses in the uncompressed tile and introducing new stresses in the compressed tile, and releasing the tile from said compression, said inward locations being such that on said release of compression inward locations remain.

3. The method of treating a substantially square tile 60 of porous fiberboard useful as ceiling tile, which tile has a face coat thereon, which comprises compressing the tile with its back on a spherically convex platen by applying a substantially planar platen and thereby substantially uniformly loading the exposable tile face, whereby during compression to deform the tile to a concave back surface corresponding to said convex platen and thereby altering the original stresses in the uncompressed tile and introducing new stresses in the compressed tile, and releasing the tile from said compression.

4. The method of treating a substantially square tile 65 of porous fiberboard useful as ceiling tile, which tile has a face coat thereon, which comprises compressing the tile with its back on a spherically convex platen by applying a heated substantially planar platen embossed with a design and thereby hot-pressing portions of the surface to

inward locations and thereby substantially uniformly loading the exposable tile face, whereby during compression to deform the tile to a concave back surface corresponding to said convex platen and thereby altering the original stresses in the uncompressed tile and introducing new stresses in the compressed tile, and releasing the tile from said compression, said inward locations being such that on said release of compression inward locations remain.

## References Cited in the file of this patent

## UNITED STATES PATENTS

|           |              |       |                |
|-----------|--------------|-------|----------------|
| 1,398,926 | Waite        | ----- | Nov. 29, 1921  |
| 1,589,898 | Reeves       | ----- | June 22, 1926  |
| 2,852,412 | Hassel       | ----- | Sept. 16, 1958 |
| 2,897,546 | Clapp et al. | ----- | Aug. 4, 1959   |